



US006023806A

# United States Patent [19]

Dumlao et al.

[11] Patent Number: 6,023,806

[45] Date of Patent: \*Feb. 15, 2000

[54] **MODULAR POLYMER MATRIX COMPOSITE SUPPORT STRUCTURE AND METHODS OF CONSTRUCTING SAME**

[75] Inventors: **Chris Dumlao**, Pleasanton; **Kristina Lauraitis**, San Jose; **Les Fisher**, Palo Alto; **Alan Miller**, Santa Cruz; **Eric Abrahamson**, Palo Alto, all of Calif.

[73] Assignee: **Martin Marietta Materials, Inc.**, Raleigh, N.C.

[\*] Notice: This patent is subject to a terminal disclaimer.

[21] Appl. No.: 08/723,098

[22] Filed: Sep. 30, 1996

[51] Int. Cl.<sup>7</sup> ..... E01D 19/12

[52] U.S. Cl. ..... 14/73; 14/74.5; 14/77.1

[58] Field of Search ..... 14/3-4, 6, 73, 14/74, 74.5, 77.1; 404/17, 18, 28, 70, 71; 52/309.1, 309.6, 783.17, 783.18, 783.19; 428/107, 112, 113, 116, 119

[56] **References Cited**

U.S. PATENT DOCUMENTS

1,754,784 4/1930 Borsodi ..... 428/119 X  
2,211,513 8/1940 Nagin .  
2,307,869 1/1943 Tench .  
2,907,417 10/1959 Doerr .

(List continued on next page.)

FOREIGN PATENT DOCUMENTS

58651 4/1941 Denmark ..... 428/119  
0 413 500 2/1991 European Pat. Off. .  
1023784 2/1958 Germany ..... 14/73  
WO 81/01807 7/1981 WIPO ..... 428/119  
WO 94/25682 11/1994 WIPO .

OTHER PUBLICATIONS

"Plastics & Composites In Construction", *Engineering News-Record*, ENR Special Advertising Section (Nov. 1995), 20 pp.

Goldstein, "Catching Up On Composites", *Civil Engineering* (Mar. 1996), pp. 47-49.

Head, "High Performance Structural Materials Advanced Composites", draft of paper to be given at the Copenhagen IABSE Conference, Copenhagen, Denmark, Jan. 1996, 18 pp.

Head, P.R., "Advanced Composites in Civil Engineering—A Critical Overview At This High Interest, Low Use Stage of Development", pp. 3-15 (El-Badry, Mamdouh, Ed., *Advanced Composite Materials in Bridges and Structures*, 2nd Annual Conference, Aug. 11-14, 1996; The Canadian Society for Civil Engineering (1996)).

(List continued on next page.)

Primary Examiner—James A. Lisehora  
Attorney, Agent, or Firm—McDermott, Will & Emery

[57] **ABSTRACT**

A load bearing support structure in the form of a traffic-bearing highway bridge including at least one modular structural section. The at least one modular structural section includes at least one beam, the beam comprising a pair of lateral flanges and a medial web between and extending below the flanges. The beam preferably has a flat floor. A load bearing deck is positioned above and supported by the flanges of the at least one beam. The beam and load bearing deck are preferably formed of a polymer matrix composite material. The beam is positioned on and supported by one of a plurality of support members. The beam has a contoured shape configured to be matingly supported by a support member having a reciprocally configured contoured shape. Alternatively, a flat or L-shape support member can be utilized. Further alternatively, the load bearing deck comprising at least one sandwich panel is suitable for applications such as barge decks, hatchcovers, and other load bearing wall applications. Methods of constructing a support structure utilizing the modular structural section and support members are also provided.

**40 Claims, 15 Drawing Sheets**



## U.S. PATENT DOCUMENTS

|           |         |                                   |
|-----------|---------|-----------------------------------|
| 3,104,194 | 9/1963  | Zahorski .                        |
| 3,112,532 | 12/1963 | Slowinski .                       |
| 3,257,764 | 6/1966  | Cripe .                           |
| 3,302,361 | 2/1967  | Oudheusden, Jr. et al. .... 14/73 |
| 3,607,592 | 9/1971  | Jenkins .                         |
| 3,708,385 | 1/1973  | Immethun ..... 428/119            |
| 3,849,237 | 11/1974 | Zetlin .                          |
| 3,906,571 | 9/1975  | Zetlin .                          |
| 4,051,289 | 9/1977  | Adamson ..... 428/113             |
| 4,084,029 | 4/1978  | Johnson et al. ..... 428/119      |
| 4,129,917 | 12/1978 | Sivachenko et al. ..... 14/73     |
| 4,177,306 | 12/1979 | Schulz et al. .                   |
| 4,185,440 | 1/1980  | Finsterwalder .                   |
| 4,186,535 | 2/1980  | Morton .                          |
| 4,223,053 | 9/1980  | Brogan .                          |
| 4,229,919 | 10/1980 | Hughes .                          |
| 4,292,364 | 9/1981  | Wesch et al. .                    |
| 4,307,140 | 12/1981 | Davis .                           |
| 4,356,678 | 11/1982 | Andrews et al. .                  |
| 4,409,274 | 10/1983 | Chaplin et al. ..... 428/112      |
| 4,416,097 | 11/1983 | Weir .                            |
| 4,467,728 | 8/1984  | Horne .                           |
| 4,525,965 | 7/1985  | Woelfel .                         |
| 4,574,108 | 3/1986  | Fakirov et al. .                  |
| 4,588,443 | 5/1986  | Bache .                           |
| 4,600,634 | 7/1986  | Langer .                          |
| 4,617,217 | 10/1986 | Michaud-Soret .                   |
| 4,629,358 | 12/1986 | Springston et al. .               |
| 4,706,319 | 11/1987 | Sivachenko et al. .               |
| 4,709,456 | 12/1987 | Iyer .                            |
| 4,788,269 | 11/1988 | Vu et al. .                       |
| 4,908,254 | 3/1990  | Fischer et al. .                  |
| 4,945,594 | 8/1990  | Tomb .                            |
| 4,976,490 | 12/1990 | Gentle .                          |
| 4,982,538 | 1/1991  | Horstketter .                     |
| 4,991,248 | 2/1991  | Allen .                           |
| 5,033,147 | 7/1991  | Svensson .                        |
| 5,052,164 | 10/1991 | Sandow ..... 52/309.1 X           |
| 5,070,668 | 12/1991 | Lieberman .                       |
| 5,179,152 | 1/1993  | Shimaoka et al. .                 |
| 5,205,098 | 4/1993  | Landis et al. .                   |
| 5,225,237 | 7/1993  | Magnani .                         |
| 5,256,223 | 10/1993 | Alberts et al. .                  |
| 5,305,568 | 4/1994  | Beckerman .                       |
| 5,309,690 | 5/1994  | Symons .                          |
| 5,417,792 | 5/1995  | Scola et al. .                    |
| 5,498,763 | 3/1996  | McGarry et al. .                  |
| 5,508,082 | 4/1996  | Ehrat et al. .                    |
| 5,508,085 | 4/1996  | Lockshaw et al. .                 |
| 5,514,444 | 5/1996  | Buyny et al. .                    |
| 5,529,808 | 6/1996  | Eguchi et al. .                   |
| 5,547,735 | 8/1996  | Roebroeks et al. .                |
| 5,585,155 | 12/1996 | Heikkila et al. .                 |
| 5,591,933 | 1/1997  | Li et al. .                       |
| 5,601,888 | 2/1997  | Fowler .                          |
| 5,601,919 | 2/1997  | Symons .                          |
| 5,612,117 | 3/1997  | Bélanger et al. .                 |

## OTHER PUBLICATIONS

Seible, F., "Advanced Composites Materials For Bridges In The 21st Century", pp. 17-30 (El-Badry, Mamdouh, Ed. Advanced Composite Materials in Bridges and Structures,

2nd Annual Conference, Aug. 11-14, 1996; The Canadian Society for Civil Engineering (1996)).

Cosenza, E., et al., "Experimental Evaluation Of Bending And Torsional Deformability Of FRP Pultruded Beams", pp. 117-124 (El-Badry, Mamdouh, Ed., Advanced Composite Materials in Bridges and Structures, 2nd Annual Conference, Aug. 11-14, 1996; The Canadian Society for Civil Engineering (1996)).

Sheard, P., et al., "Eurocrete—Using Advanced Composites To Reinforce Durable Concrete Structures", pp. 159-164 (El-Badry, Mamdouh, Ed., Advanced Composite Materials in Bridges and Structures, 2nd Annual Conference, Aug. 11-14, 1996; The Canadian Society for Civil Engineering (1996)).

Aref, A., et al., "Design and Analysis Procedures For A Novel Fiber Reinforced Plastic Bridge Deck", pp. 743-750 (El-Badry, Mamdouh, Ed., Advanced Composite Materials in Bridges and Structures, 2nd Annual Conference, Aug. 11-14, 1996; The Canadian Society for Civil Engineering (1996)).

Karbhari, V.M., "Fiber Reinforced Composite Decks For Infrastructure Renewal", pp. 759-766 (El-Badry, Mamdouh, Ed., Advanced Composite Materials in Bridges and Structures, 2nd Annual Conference, Aug. 11-14, 1996; The Canadian Society for Civil Engineering (1996)).

Johansen, G. Eric, et al., "Design And Construction Of Two FRP Pedestrian Bridges In Haleakala National Park, Maui, Hawaii", pp. 975-982 (El-Badry, Mamdouh, Ed., Advanced Composite Materials in Bridges and Structures, 2nd Annual Conference, Aug. 11-14, 1996; The Canadian Society for Civil Engineering (1996)).

Johansen et al., "Design of an Advanced Composite Material Space Frame System", pp. 1-9 of Session 7-B [Composites Institute's 51st Annual Conference & Expo '96, Feb. 5-7, 1996; SPI Composites Institute (1996)].

Gentry, "Application and Performance of Sandwich Panel Composites for Transportation Facilities", pp. 1-6 of Session 7-C [Composites Institute's 51st Annual Conference & Expo '96, Feb. 5-7, 1996; SPI Composites Institute (1996)].

Johansen et al., "Advanced Composite Material Support Frames: An Evaluation of the Bow Meadow Bridge at Lake Crescent, WA", pp. 1-9 of Session 7-D [Composites Institute's 51st Annual Conference & Expo '96, Feb. 5-7, 1996; SPI Composites Institute (1996)].

Barbero et al., "Stiffening of Steel Stringer Bridges with Carbon Fiber Reinforced Plastics for Improved Bridge Rating", pp. 1-3 of Session 7-E [Composites Institute's 51st Annual Conference & Expo '96, Feb. 5-7, 1996; SPI Composites Institute (1996)].

Meteer, "Designing Structural Sandwich Composites", pp. 1-6 of Session 8-D [Composites Institute's 51st Annual Conference & Expo '96, Feb. 5-7, 1996; SPI Composites Institute (1996)].

Churchman, Allan E., "Design Considerations for Advanced Composite Materials", 7 pp. [Fiberglass-Composite Bridges Seminar, 13th Annual Bridge Conference and Exhibition (Jun. 3, 1996)].

Witcher, Daniel A., "Processing and Fabricating FRP Composites For Bridge Structures", 9 pp. [Fiberglass-Composite Bridges Seminar, 13th Annual Bridge Conference and Exhibition (Jun. 3, 1996)].

Busel, John, Ed., *FRP Composites in Construction Applications, A Profile in Progress*, SPI Composites Institute (Nov. 1995), pp. 11–13, 15–16, 19–20, 49, 51–52, 58, 61, 73–74, 76–78, and 81.

“Tom’s Creek Bridge Rehabilitation & Field Composite Durability Study”, Virginia Tech; Virginia Transportation Research Council; Morrison Molded Fiber Glass (1996), 2 pages.

*Standard Specifications for Highway Bridges*, 15th Edition (1992), American Association of State Highway and Transportation Officials, Inc., Washington, D.C., 13 pp.

*Introduction to Composites*, Third Edition, The Composites Institute of the Society of the Plastics Industry, Inc. (released Jan., 1995), pp. 67–84.





FIG. 3



FIG. 4



FIG. 5



FIG. 6



FIG. 7



FIG. 8



FIG. 9



FIG. 10





FIG. 12



FIG. 13



FIG. 14



FIG. 15



FIG. 16



FIG. 17



FIG. 18



FIG. 19

**MODULAR POLYMER MATRIX  
COMPOSITE SUPPORT STRUCTURE AND  
METHODS OF CONSTRUCTING SAME**

**FIELD OF THE INVENTION**

This invention relates to support structures such as bridges, piers, docks, load bearing decking applications, such as hulls and decks of barges, and load bearing walls. More particularly, this invention relates to a modular composite load bearing support structure including a polymer matrix composite modular structural section for use in constructing bridges and other load bearing structures and components.

**BACKGROUND OF THE INVENTION**

Space spanning structures such as bridges, docks, piers, load bearing walls, hulls, and decks which have provided a span across bodies of water or separations of land and water and/or open voids have long been made of materials such as concrete, steel or wood. Concrete has been used in building bridges, and other structures including the columns, decks, and beams which support these structures.

Such concrete structures are typically constructed with the concrete poured in situ as well as using some preformed components precast into structural components, such as supports, and transported to the site of the construction.

Constructing such concrete structures in situ requires hauling building materials and heavy equipment and pouring and casting the components on site. This process of construction involves a long construction time and is generally costly, time consuming, subject to delay due to weather and environmental conditions, and disruptive to existing traffic patterns when constructing a bridge on an existing roadway.

On the other hand, pre-cast concrete structural components are extremely heavy and bulky and are typically costly and difficult to transport to the site of construction due in part to their bulkiness and heavy weight. Although construction time is shortened compared to construction with concrete poured in situ, extensive construction time with resulting delays is still a factor. Bridge construction with such precast forms is particularly difficult, if not impossible, in remote or difficult terrain such as mountains or jungle areas in which numerous bridges are constructed.

In addition to construction and shipping difficulties with concrete bridge structures, the low tensile strength of concrete can result in failures in concrete bridge structures, particularly in the surface of bridge components. Reinforcement is often required in such concrete structures when subjected to large loads such as in highway bridges. Steel and other materials have been used to reinforce concrete structures. If not properly installed, such reinforcements cause cracking and failure in the reinforced concrete, thereby weakening the entire structure. Further, the inherent hollow spaces which exist in concrete are highly subject to environmental degradation. Also, poor workmanship often contributes to the rate of deterioration.

In addition to concrete, steel also has been widely used by itself as a building material for structural components in structures such as bridges, barge decks, vessel hulls, and load bearing walls. While having certain desirable strength properties, steel is quite heavy and costly to ship and can share construction difficulties with concrete as described.

Steel and concrete are also susceptible to corrosive elements, such as water, salt water and agents present in the environment such as acid rain, road salts, chemicals, oxygen

and the like. Environmental exposure of concrete structures leads to pitting and spalling in concrete and thereby results in severe cracking and a significant decrease in strength in the concrete structure. Steel is likewise susceptible to corrosion, such as rust, by chemical attack. The rusting of steel weakens the steel, transferring tensile load to the concrete, thereby cracking the structure. The rusting of steel in stand alone applications requires ongoing maintenance, and after a period of time corrosion can result in failure of the structure. The planned life of steel structures is likewise reduced by rust.

The susceptibility to environmental attack of steel requires costly and frequent maintenance and preventative measures such as painting and surface treatments. In completed structures, such painting and surface treatment is often dangerous and time consuming, as workers are forced to treat the steel components in situ while exposed to dangerous conditions such as road traffic, wind, rain, lightning, sun and the like. The susceptibility of steel to environmental attack also requires the use of costly alloys in certain applications.

Wood has been another long-time building material for bridges and other structures. Wood, like concrete and steel, is also susceptible to environmental attack, especially rot from weather and termites. In such environments, wood encounters a drastic reduction in strength which compromises the integrity of the structure. Moreover, wood undergoes accelerated deterioration in structures in marine environments.

Along with environmental attack, deterioration and damage to bridges and other traffic and load bearing structures occurs as a result of heavy use. Traffic bearing structures encounter repeated heavy loads of moving vehicles, stresses from wind, earthquakes and the like which cause deterioration of the materials and structure.

For the reasons described above, the United States Department of Transportation "Bridge Inventory" reflects several hundred thousand structures, approximately forty percent of bridges in the United States, made from concrete, steel and wood are poorly maintained and in need of rehabilitation in the United States. The same is believed to be true for other nations.

The associated repairs for such structures are extremely costly and difficult to undertake. Steel, concrete and wood structures need welding, reinforcement and replacement. Decks and hulls of structures in marine environments rust, requiring constant maintenance and vigilance. In numerous instances, these necessary repairs are not feasible or economically justifiable and cannot be undertaken, and thereby require the replacement of the structure. Further, in developing areas where infrastructures are in need of development or improvement, those constructing bridges and other such structures utilizing concrete, steel and wood face unique difficulties. Difficulty and high cost has been associated with transporting materials to remote locations to construct bridges with concrete and steel. This process is more costly in marine environments where repairs require costly dry-docking or transport of materials. Also, the degree of labor and skill is very high using traditional building materials and methods.

Further, traditional construction methods have generally taken long time periods and required large equipment and massive labor costs. Thus, development and repair of infrastructures throughout the world has been hampered or even precluded due to the cost and difficulty of construction. Further, in areas where structures have been damaged due to

deterioration or destroyed by natural disaster such as earthquake, hurricane, or tornado, repair can be disruptive to traffic or use of the bridge or structure or even delayed or prevented due to construction costs.

In addressing the limitations of existing concrete, wood and steel structures, some fiber reinforced polymer composite materials have been explored for use in constructing parts of bridges including foot traffic bridges, piers, and decks and hulls of some small vessels. Fiber reinforced polymers have been investigated for incorporation into foot bridges and some other structural uses such as houses, catwalks, and skyscraper towers. These composite materials have been utilized, in conjunction with, and as an alternative to, steel, wood or concrete due to their high strength, light weight and highly corrosion resistant properties. However, it is believed that construction of traffic bridges, marine decking systems, and other load bearing applications built with polymer matrix composite materials have not been widely implemented due to extremely high costs of materials and uncertain performance, including doubts about long term durability and maintenance.

As cost is significant in the bridge construction industry, such materials have not been considered feasible alternatives for many load bearing traffic bridge designs. For example, high performance composites made with relatively expensive carbon fibers have frequently been eliminated by cost considerations. These same cost considerations have inhibited the use of composite materials in decking and hull applications.

In investigating providing structural components made from fiber reinforced polymer composite materials, components structures from prior materials such as steel, concrete and wood have been investigated. Steel trusses and supports have utilized triangular shapes welded together. Providing triangular structural components with composite materials has presented problems of failure in the resin bonded nodes of the triangular shape. Therefore a modular structural composite component for structural supports is needed which overcomes this problem.

In view of the problems associated with bridges and other structures formed of steel, concrete, and wood described herein, there remains a need for a bridge or like support structure with the following characteristics: light-weight; low cost, pre-manufactured; constructed of structural modular components; easily shipped, constructed, and repaired without requiring extensive heavy machinery; and resistant to corrosion and environmental attack, even without surface treatment. There is also a need for a support structure which can provide the structural strength and stiffness for constructing a highway bridge or similar support structure.

#### SUMMARY OF THE INVENTION

In view of the foregoing, it is therefore an object of the present invention to provide a load bearing support structure suitable for a highway bridge structure or decking system in marine and other construction applications, constructed of modular structural sections formed of a lightweight, high performance, environmentally resistant material.

It is another object of the invention to provide a support structure such as a highway bridge structure which satisfies accepted design, performance, safety and durability criteria for traffic bearing bridges of various types.

It is another object of the present invention to provide such a support structure in the form of a traffic-bearing bridge in a variety of designs and sizes constructed of modular structural sections which can be constructed quickly, cost-effectively and with limited heavy machinery and labor.

It is also an object of the present invention to provide such a support structure, such as a bridge, constructed of components which can easily and cost-effectively be shipped to the site of construction as a complete kit.

It is likewise an object of the present invention to provide a support structure including a modular structural section which can be utilized to quickly repair or replace a damaged bridge, bridge section or like support structure.

It is another object of the present invention to provide a load bearing support structure including a modular structural section which can be used in decking, hull, and wall applications.

It is still another object of the invention to provide a support structure or bridge which requires minimal maintenance and upkeep with respect to surface treatment or painting.

These and other objects, advantages and features are satisfied by the present invention, which is directed to a polymer matrix composite modular load bearing support structure described herein for exemplary purposes in the form of a highway bridge. The support structure of the present invention includes a plurality of support members and at least one modular structural section positioned on and supported by the support members. The modular structural section is preferably formed of a polymer matrix composite.

The modular structural section includes at least one beam and a load bearing deck positioned above and supported by the beam. The at least one beam includes a pair of lateral flanges and a medial web between and extending below the flanges. In one embodiment, the flanges and the web have a predetermined shape which matingly contacts surfaces of support means which also have a predetermined contoured shape. The flanges and web are positioned on and supported by the contoured shaped support means. In a preferred embodiment, the lateral flanges and the web also preferably form a U-shaped cross-section having a generally flat floor in the medial portion.

In an alternative embodiment, the flat floor of the elongate support can be positioned on and supported by support means having a surface having a generally flat portion preferably a support member or abutment with a flat cap portion.

In a further alternative embodiment, the support means in the form of a support member or abutment can be provided having a surface having a horizontal cap surface perpendicular to a vertical wall surface forming an L-shape surface for supporting the beam and deck of the modular structural section. The beam is preferably positioned, in this embodiment with the flat floor positioned above the horizontal cap surface and the end edge of the web and flanges of the modular structural section positioned flush with the vertical wall surface.

In all of these embodiments, the polymer matrix composite support structure of the present invention can provide a support surface sufficient to support vehicular traffic and to conform to established design and performance criteria.

Alternatively, the modular structural section, including the load-bearing deck and beam, can be used in constructing other support structures including space-spanning support structures. Further, the load bearing deck can also be used as a stand alone decking, hull, or wall system which can be integrated into a marine or construction system. The load bearing decking system can be utilized in numerous applications where load bearing decking, hulls and walls are required.

The support structure also reduces tooling and fabrication costs. The support structure is easy to construct utilizing

prefabricated components which are individually lightweight, yet structurally sound when utilized in combination. The modularity of the components enhances portability, facilitates pre-assembly and final positioning with light load equipment, and reduces the cost of shipping and handling the structural components. The support structure allows for easy construction of structures such as, but not limited to, bridges, marine decking applications and other construction and transportation applications.

The load bearing deck of the modular structural section also includes at least one sandwich panel including an upper surface, a lower surface and a core. The core includes a plurality of substantially hollow, elongated core members positioned between the upper surface and the lower surface. Each of the elongate core members includes a pair of side walls. The side walls can be formed and disposed in a variety of shapes angles with respect to the upper and lower walls. Each core member has side walls positioned generally adjacent to a side wall of an adjacent core member. The upper and lower surfaces of the sandwich panel are preferably an upper facesheet and lower facesheet formed of a polymer matrix composite material. In one embodiment, the upper and lower facesheets are formed of polymer matrix composite arranged in a hybrid of alternating layers including carbon and E-glass fibers in vinylester or polyester resin.

In one embodiment of the bridge described herein for a 30 foot span highway bridge, the individual components including the beams and the sandwich panels for the deck of the modular structural section each weigh less than 3600 pounds. Being constructed of a number of modular structural sections including components manufactured from polymer matrix composites, instead of concrete, steel and wood, the bridge has individual modular components which are fault tolerant in manufacture, as twisting and small warpage can be corrected at assembly. These properties of the bridge components decrease the cost of manufacture and assembly for the bridge. These components, including lightweight modular structural sections manufactured under controlled conditions, also allow for low cost assembly of a number of applications, such as marine structures, including the various applications described herein.

Another aspect of the present invention is a method of constructing a support structure such as highway bridge. The method comprises the following steps. First, a plurality of spaced-apart support members having a predetermined shape, for example a contoured shape, are provided. Next, a modular structural section is positioned on the plurality of spaced-apart support members. In one embodiment, the elongate support members of the modular structural section have a contoured shape which matably joins with and is supported on the contoured shape of support members. The modular structural section and the support members are then in various embodiment connected.

In one embodiment, the modular structural section is positioned by: first, positioning the beam having a contoured shape upon adjacent of the support members having a contoured shape for matably joining with and supporting the beam; then positioning the load bearing deck upon the beam, then connecting the at least one beam with the deck.

In another embodiment, a load bearing pad is first positioned on a flat cap portion of a support member. Then, the modular structural section is positioned on the load bearing pad with the flat floor of the beam positioned on the load bearing pad.

The methods of the present invention provide significantly reduced time, labor and cost as compared to conven-

tional methods of bridge and support structure construction utilizing concrete, wood and metal structures.

#### BRIEF DESCRIPTION OF THE DRAWINGS

FIG. 1 is a perspective view of a load bearing support structure in the form of a traffic highway bridge according to the present invention and a truck traveling thereon.

FIG. 2 is a cutaway partial perspective view of a modular structural section of the bridge according to the present invention.

FIG. 3 is an exploded view of a sandwich panel deck of FIG. 2 having trapezoidal core members.

FIG. 4 is an exploded perspective view of a plurality of contoured beams positioned on contoured support members of the bridge of FIG. 2.

FIG. 5 is an exploded perspective view of the sandwich panel deck being positioned on the beams of the bridge of FIG. 2.

FIG. 6 is an end view of the modular structural section of the bridge of FIG. 2 showing a support diaphragm positioned in the end thereof.

FIG. 7 is an enlarged cross-sectional view of adjacent panels of the sandwich deck of FIG. 2 being joined with a key lock.

FIG. 8 is a cross-section, exploded view of the facesheets of the modular structural section.

FIG. 9 is a perspective view of an alternative embodiment of a load bearing support structure in the form of a traffic highway bridge having a flat support member according to the present invention and a truck traveling thereon.

FIG. 10 is an exploded partial perspective view of a modular structural section of the bridge of FIG. 9 according to the present invention.

FIG. 11 is a perspective view of an alternative embodiment of a load bearing support structure in the form of a traffic highway bridge having a L-shape support member according to the present invention and a truck traveling thereon.

FIG. 12 is an exploded partial perspective view of a modular structural section of the bridge of FIG. 11 according to the present invention.

FIG. 13 is a perspective view of an alternative embodiment of a load bearing support structure in the form of a traffic highway bridge having a flat support member according to the present invention and a truck traveling thereon.

FIG. 14 is an exploded partial perspective view of a modular structural section of the bridge of FIG. 13 according to the present invention.

FIG. 15 is a perspective view of an alternative embodiment of a load bearing support structure in the form of a traffic highway bridge having a L-shape support member according to the present invention and a truck traveling thereon.

FIG. 16 is an exploded partial perspective view of a modular structural section of the bridge of FIG. 11 according to the present invention.

FIG. 17 is an exploded perspective view of the modular structural section of the bridge of FIG. 2 showing an alternative embodiment of support diaphragms positioned in the end thereof.

FIG. 18 is an exploded perspective view of the modular structural section of the bridge of FIG. 2 showing an alternative embodiment of a support diaphragm positioned on the end thereof.

FIG. 19 is an exploded perspective view of the modular structural section of the bridge of FIG. 2 showing an alternative embodiment of a support diaphragm positioned on the end thereof.

#### DETAILED DESCRIPTION OF THE PREFERRED EMBODIMENTS

The present invention now will be described more fully hereinafter with reference to the accompanying drawings, in which preferred embodiments of the invention are shown. This invention can, however, be embodied in many different forms and should not be construed as limited to the embodiments set forth herein; rather, Applicant provides these embodiments so that this disclosure will be thorough and complete, and will fully convey the scope of the invention to those skilled in the art.

Referring now to the figures, a modular composite support structure in the form of a bridge structure 20 according to the present invention is shown. This embodiment of the bridge 20 is designed to exceed standards for bridge construction such as American Association of State Highway and Transportation Officials (AASHTO) standards. The AASHTO standards include design and performance criteria for highway bridge structures. The AASHTO standards are published in "Standard Specifications for Highway Bridges," American Association of State Highway and Transportation Officials, Inc., (15th Ed., 1992) which is hereby incorporated by reference in its entirety. Support structures, including bridges, of the present invention can be constructed which meet other structural, design and performance criteria for other types of bridges, construction and transportation support structures, and other applications including, but not limited to, road bearing decking systems and marine applications.

The support structure is described with reference to a traffic-bearing highway bridge herein. As shown in FIGS. 1 and 2, the bridge 20 is a simply-supported highway bridge capable of withstanding loads from highway traffic such as the truck T. The bridge 20 has a span defined by the length of the bridge 20 in the direction of travel of truck T. The bridge 20 comprises a modular structural section 30 including a deck 32 and beams 50, 50', 50" and a deck 32 supported on and connected with the beams 50, 50', 50" (FIG. 2). The modular structural section 30 is supported on support members 22.

In addition to a simply-supported bridge, alternatively, the bridge including the modular structural section according to the present invention can be provided in other types of bridges including lift span bridges, cantilever bridges, cable suspension bridges, suspension bridges and bridges across open spaces in industrial settings. Various spans of bridges can be provided including, but not limited to, short, medium and long span bridges. The bridge technology can also be supplied for bridges other than highway bridges such as foot bridges and bridge spans across open spaces in industrial settings. Other space spanning support structures can also be constructed in a similar manner to that indicated including, but not limited to, bridge component maintenance (replacement decking, column/beam supports, abutments, abutment forms and wraps), marine structures (walkways, decking (small/large scale)), load bearing decking systems, drill platforms, hatch covers, parking decks, piers and fender systems, docks, catwalks, super-structure in processing and plants with corrosive environments and the like which provide an elevated support surface over a span, rail cross ties, space frame structures (conveyors and structural

supports) and emission stack liners. Other structures such as railroad cars, shipping containers, over-the-road trailers, rail cars, barges and vessel hulls could also be constructed in a similar manner to that indicated. The components of the bridge 20, including the modular structural section 30 and constituent deck 32 and beam 50, as described herein, can also be provided, individually and in combination, in such other support structures as described.

The support members 22, in this embodiment, have a predetermined contoured shape configured to matably contact and join with the predetermined shape of the beams 50, 50', 50". The support members each have a plurality of spaced-apart peak portions 23 and a plurality of spaced apart trough portions 25 positioned adjacent to and between said peak portions 23 (FIG. 2). The peak portions 23 and the trough portions 25 are generally flat to matably contact and support the beams 50, 50', 50". The column peak portions 23 and the trough portions 25 are arranged and spaced apart a predetermined distance to facilitate supporting the beams 50, 50', 50".

Each of the beams 50, 50', 50" have flanges 51, 52 which are positioned on the peak portions 23 of the support members 22. Each of the beams 50, 50', 50" also have a medial web 53 between and extending below the flanges 51, 52. As shown in FIGS. 5 and 6 the medial web 53 includes an inclined sidewall 54 and a generally flat floor 68. The trough portion 25 of the support members 22 supports the medial web 53 including the inclined side walls 54 and the flat floor 68. In the bridge 20 of FIG. 1, the support members are positioned at opposite ends 55, 56 of the beams 50. Alternatively, the beams 50 can be supported by support members at intermediate positions along the length of the beam 50.

The support members can be provided in various other shapes and configurations, including other contoured shapes which are configured to correspond to the shape of the beams 50. In other alternative embodiments, the support members or other support means can include the supports of an existing bridge replaced by the bridge 20 of the present invention. Alternative embodiments of the support members can be formed of other materials such as composite materials, steel, wood or other materials. Further, alternative embodiments of the support members are shown in applications to the common assignee of this application entitled "MODULAR COMPOSITE SUPPORT STRUCTURE AND METHODS OF CONSTRUCTING SAME", filed concurrently, Ser. No. 08/723,359, (Attorney Docket No. 8637-5) and entitled "MODULAR COMPOSITE SUPPORT STRUCTURE AND METHODS OF CONSTRUCTING SAME", filed concurrently, Ser. No. 08/723,109, 50 (Attorney Docket No. 8637-88) (hereinafter "Modular Composite Support Structure applications") the disclosure of which is hereby incorporated by reference in its entirety. Additional support means depend on the type of support structure constructed.

In the embodiment of FIGS. 1-5 and 7, the support members 22, and the modular structural section 30, including the deck 32 and beams 50 are formed of a polymer matrix composite comprising reinforcing fibers and a polymer resin. Suitable reinforcing fibers include glass fibers, including but not limited to E-glass and S-glass, as well as carbon, metal, high modulus organic fibers (e.g., aromatic polyamides, polybenzimidazoles, and aromatic polyimides), and other organic fibers (e.g., polyethylene and nylon). Blends and hybrids of the various fibers can be used. Other suitable composite materials could be utilized including whiskers and fibers such as boron, aluminum silicate and basalt.

The resin material in the support members 22 and the modular structural section 30, including the deck 32 and the beams 50, 50', 50", are preferably a thermosetting resin, and more preferably a vinyl ester resin. The term "thermosetting" as used herein refers to resins which irreversibly solidify or "set" when completely cured. Useful thermosetting resins include unsaturated polyester resins, phenolic resins, vinyl ester resins, polyurethanes, and the like, and mixtures and blends thereof. The thermosetting resins useful in the present invention may be used alone or mixed with other thermosetting or thermoplastic resins. Exemplary other thermosetting resins include epoxies. Exemplary thermoplastic resins include polyvinylacetate, styrene-butadiene copolymers, polymethylmethacrylate, polystyrene, cellulose acetatebutyrate, saturated polyesters, urethane-extended saturated polyesters, methacrylate copolymers and the like.

Polymer matrix composites can, through the selective mixing and orientation of fibers, resins and material forms, be tailored to provide mechanical properties as needed. These polymer matrix composite materials possess high specific strength, high specific stiffness and excellent corrosion resistance. In the embodiment shown in FIGS. 1-5 and 7, a polymer matrix composite material of the type commonly referred to as a fiberglass reinforced polymer (FRP) or sometimes, as glass fiber reinforced polymer (GFRP) is utilized in the support members 22, deck 32 and the beams 50, 50', 50". The reinforcing fibers of the support members 22 and the modular structural section 30, including the deck 32 and the beams 50, 50', 50", are glass fibers, particularly E-glass fibers, and the resin is a vinyester resin. Glass fibers are readily available and low in cost. E-glass fibers have a tensile strength of approximately 3450 MPa (practical). Higher tensile strengths can alternatively be accomplished with S-glass fibers having a tensile strength of approximately 4600 MPa (practical). Polymer matrix composite materials, such as a fiber reinforced polymer formed of E-glass and a vinyester resin have exceptionally high strength, good electrical resistivity, weather and corrosion-resistance, low thermal conductivity, and low flammability.

The support members 22 are preferably formed of fiber-glass fibers in a vinyester resin. Alternatively, the support members 22 can be formed of other polymer matrix composite materials, as described herein, or other materials such as concrete in precast footings or poured in situ, steel, wood or other building materials. An alternative embodiment of the support member 122 shown in FIG. 6 is a pre-cast concrete footing having the contoured shape of the previously described support member 22.

#### The Deck

In the bridge 20 including the modular structural section 30 shown in FIGS. 1-2, the deck 32 includes three sandwich panels 34, 34' 34". Alternatively, any number of panels can be utilized in a deck depending on the length of the desired span. As shown in FIG. 3, each sandwich panel 34 comprises an upper surface shown as an upper facesheet 35, a lower surface shown as a lower facesheet 40 and a core 45 including a plurality of elongate core members 46.

The core members 46 are shown as hollow tubes of trapezoidal cross-section (FIGS. 2, 3 and 7). Each of the trapezoidal tubes 46 includes a pair of side walls 48, 49. One of the side walls 48 is disposed at an oblique angle  $\alpha$  to one of the upper and lower facesheets 35, 40 such that the side walls 48, 49 and the upper wall 64 and lower wall 65, when viewed in cross-section, define a polygonal shape such as a trapezoidal cross-section (FIG. 3). The oblique angle  $\alpha$  of the side wall 48 with respect to the upper wall 64 is preferably

about 45°, but angles between about 30° and 45° can be provided in alternative embodiments. Each tube 46 has a side wall 48 positioned generally adjacent to a side wall 48' of an adjacent tube 46' (FIG. 3). Alternatively, the tubes 46 could be aligned in other configurations such as having a space between adjacent side walls.

The side walls 48, 48' disposed at an oblique angle  $\alpha$  provide transverse shear stiffness for the deck core 45. This increases the transverse bending stiffness of the overall deck 32. The sidewall 48 shown at the preferred 45° angle  $\alpha$  provides the highest bending stiffness. The trapezoidal tubes 46 also preferably have a vertical side wall 49 positioned between adjacent diagonal side walls 48, 48'. The vertical sidewall 49 provides structural support for localized loads subjected on the deck 32 to prevent excessive deflection of the top facesheet 35 along the span between the intersection of the diagonal walls 48, 48' and the upper facesheet 35.

Thus, the shape including the angled side wall 48 of the trapezoidal tube 46 provides stiffness across the cross-section of the tube 46. An adjacent tube 46' includes a side wall 48' angled in an opposite orientation between the upper and lower walls 64, 65 from the adjacent angled side wall 48. Providing side walls 48, 49 at varying orientations preserves the mathematical symmetry of the cross-section of the tubes 46. When normalized by weight, the trapezoidal tube 46 with at least a 45° angle between the sidewall 48 and the upper wall 64 and the lower wall 65 has a transverse shear stiffness 2.6 times that of a tube with a square cross-section. Alternatively, for a tube with an oblique angle  $\alpha$  of about 30°, the transverse shear stiffness is 2.2 times that of a tube with a square shaped cross-section.

The span between the diagonal side walls 48, 48' and the vertical sidewall 49 can be provided in a variety of predetermined distances. A variety of sizes, shapes and configurations of the elongate core members can be provided. Various other polygonal cross-sectional shapes can also be employed, such as quadrilaterals, parallelograms, other trapezoids, pentagons, and the like. Alternative embodiments to the tubes 46 can be seen in the related Modular Composite Support Structure applications referenced previously.

As explained, adjacent tubes 46 of the core 45 have adjacent side walls 48, 48' aligned with one another (FIG. 3). The elongate tubes 46 extend in their lengthwise direction preferably in the direction of the span of the bridge (FIG. 1). Alternatively, depending on design load parameters, the tube 46 can be positioned to extend transverse to the direction of travel as seen in the commonly assigned "Modular Composite Support Structure" application referenced previously. Further, alternatively, tubes and other polygonal core members of a variety of lengths and cross-sectional heights and width dimensions can be provided in forming a deck of the modular structural section according to the present invention.

The tubes 46 are also preferably formed of a polymer matrix composite material comprising reinforcing fibers and a polymer resin. Suitable materials are the same polymer matrix composite materials as previously discussed herein, the discussion is hereby incorporated by reference. The tubes 46, are most preferably E-glass fibers in a vinyester resin (FIG. 3).

The tubes 46 can be fabricated by pultrusion, hand lay-up or other suitable methods including resin transfer molding (RTM), vacuum curing and filament winding, automated layup methods and other methods known to one of skill in the art of composite fabrication and are therefore not

## 11

described in detail herein. The details of these methods are discussed in *Engineered Materials Handbook*, Composites, Vol. 1, ASM International (1993).

When fabricating by hand lay-up, the tubes 46 can be fabricated by bonding a pair of components (not shown). One component includes the vertical side wall 49 and a portion of the upper wall 64 and lower wall 65. The other component includes the angled side wall 48 and the respective remaining portions of the upper wall 64 and lower wall 65. The upper and lower walls 64, 65 are bonded with an adhesive along the upper wall 64 and lower wall 65 where stresses are reduced.

It is believed that such forming overcomes the problem of node failure experienced in forming triangular shapes with composite materials. In a triangular section, the members behave as a pinned truss. Such a truss system transfers load directly through the vertex. To do so the truss encounters large amounts of interlaminar shear and tensile stresses. The trapezoidal tube 46 does not experience forces at a vertex such as those in a triangular section. The trapezoidal section of the tube 46 requires that the load be carried partially by bending the cross-section. Such bending relieves the interlaminar stresses resulting in a higher load carrying capacity.

Also, as described above, the sandwich panels 34 each also have an upper surface shown as an upper facesheet 35 and a lower surface shown as facesheet 40 (FIG. 3). The tubes 46 are sandwiched between a lower surface 36 of the upper facesheet 35 and the upper surface 41 of the lower facesheet 40. As seen in FIG. 3, the lower face sheet 40 and the upper face sheet 35 are sheets preferably formed of polymer matrix composite materials as described herein.

Having fabricated the upper and lower facesheets 35, 40 as described herein, the lower surface 36 of the upper face sheet 35 is preferably laminated or adhered to the upper surface 47 of the tubes 46 by a resin 26 and/or other bonding means and joined with the tubes 46 by mechanical or fastening means including, but not limited to, bolts or screws. Likewise, the upper surface 41 of the lower facesheet 40 is preferably laminated to the lower surface 27 of the tubes 46 by resin 26 or other bonding means and joined with the tubes 46 by mechanical fastening means including, but not limited to, bolts or screws.

The core 45, including the tubes 46, and the upper and lower facesheets 35, 40, can be alternatively joined with fasteners alone, including bolts and screws, or by adhesives or other bonding means alone. Suitable adhesives include room temperature cure epoxies and silicones and the like. Further, alternatively, the tubes could be provided integrally formed as a unitary structural component with an upper and lower surface such as a facesheet by pultrusion or other suitable forming methods.

As described, the sandwich panels 34, 34', 34" of the deck 32, being formed of polymer matrix composite material, provide high through thickness, stiffness and strength to resist localized wheel loads of vehicles traveling over the bridge according to regulations such as those promulgated by AASHTO.

In the deck shown in FIGS. 1-5 and 7-8, the upper and lower facesheets 35, 40 are hand laid of polymer matrix composite material. Alternatively, the facesheets 35, 40 can be fabricated using automated layup methods. The upper and lower facesheets 35, 40 are each formed of a plurality of substrate layers 61, 62 (in FIG. 8). Alternating layers of the substrate layers of the facesheets 35, 40 are preferably formed of different reinforcing fibers and a polymer resin.

Each of the facesheets 35, 40 shown in the embodiment of the deck 32 of FIG. 3 are formed of a hybrid of glass and

## 12

carbon fibers, both with vinylester or alternatively polymer resin. The facesheets 35, 40 each have an outer layer 60 formed of quasi-isotropic E-glass and a vinylester and an adjacent layer 61 formed of graphite and vinylester (FIG. 8). 5 The layers then alternate between E-glass 62, 62' and carbon 61' as shown in FIG. 8.

The outer layers 60, 63 forming the upper and lower surfaces of each facesheet 35, 40 are each formed of E-glass to provide impact resistance. The layup was determined with 10 a percentage of graphite having the same stiffness as an all E-glass and vinylester. The facesheets 35, 40 have a layup of approximately 42 per cent graphite and 58 percent E-glass. Alternatively, other types and combinations of composite materials can be used to fabricate the upper and lower 15 facesheets 35, 40 developing on the design criteria. For example, facesheets 35, 40 formed of all glass fibers can be provided in alternative embodiments.

The quasi-isotropic layup of the upper and lower facesheets 35, 40 prevent warping from non-uniform shrinkage 20 during fabrication. The orientation of the facesheets also provides a nearly uniform stiffness in all directions of the facesheets 35, 40.

Alternatively, other types of composite materials, with 25 varying orientations, can be used to fabricate the upper and lower facesheets 35, 40. For example, alternatively, the facesheets can be formed with orientations other than quasi-isotropic layup. Alternative configurations and compositions of facesheets 35, 40 can be seen in the commonly assigned 30 Modular Composite Support Structure applications referenced previously.

The upper and lower facesheets 35, 40 are fabricated in the present embodiment by the following steps. First, the lower facesheets 40 and upper facesheets 35 are fabricated by hand layup using rolls of knitted quasi-isotropic fabric. 35 The fibers of the upper and lower facesheets 35, 40 are given a predetermined orientation such as described depending on the desired properties.

While the upper and lower facesheets 35, 40, are fabricated using a hand-layup process, the core 45 including the 40 facesheets 35, 40 can alternatively be fabricated by other methods such as pultrusion, resin transfer molding (RTM), vacuum curing and filament winding and other methods known to one of skill in the art of composite fabrication, which, therefore, are not discussed in detail herein. Further, facesheets and core members alternatively can be fabricated 45 as a single component such as by pultruding a single sandwich panel having an upper and lower facesheet and a core of tubes.

As shown in FIG. 3, a single upper face sheet 35 and a 50 single lower face sheet 40 can be adhered to a plurality of tubes. Alternatively, any number of facesheets and any number of tubes can be connected to form the sandwich panel of a deck for a modular structural section. Also, 55 alternatively, various sizes and configurations of facesheets and cores can be provided to accommodate various applications. The resulting deck 32 is provided as a unitary structural component which can be used by itself or as a component of a modular structural section 30 for thereby 60 constructing a support structure including a bridge or other structure therefrom. The deck 32 can be utilized in other structural applications as described herein.

As shown in FIGS. 1 and 7, the three sandwich panels 34, 34', 34" are joined at adjacent side edges 33, 33', 33" to form 65 a planar deck surface 29. The deck 32 is positioned generally above and coextensively with upper surfaces 57, 58 of the flanges 51, 52 of the beams 50 (FIGS. 1 and 5).

Each sandwich panel 34 contains a C-channel 39 at each end 44 for joining adjacent sandwich panels 34, 34' in forming the deck 32. As shown in FIG. 7, an internal shear key lock 67 is inserted into adjacent C-channels 39, 39' to join adjacent sandwich panels 34, 34'. The shear key lock 67 is preferably formed of a bulk polymer material including, but not limited to, or polymer concrete mix. Such a shear key lock 67 formed of a polymer is preferred due to its chemical and corrosive resistant properties. Alternatively, the shear key lock 67 can be formed of various other materials such as wood, concrete, or metal.

The shear key lock 67 is bonded with the sandwich panels 34, 34' by an adhesive such as room temperature cure epoxy adhesive or other bonding means. Alternatively, the shear key lock 67 can be fastened with fasteners including bolts and screws, and the like.

Other methods of joining adjacent sandwich panels to form a deck could be utilized including, but not limited to, plane joints with external reinforcement plates on the upper and lower surface of the sandwich panels, recessed splice joints with reinforcing plates, externally trapped joints with sandwich panels joined in a dual connector, match fitting joints, and lap splice joints. These joints and joining methods are known to one of ordinary skill in the art and, therefore, are not discussed in detail herein.

#### The Beam

Referring back to FIGS. 1 and 2, the modular structural section 30 also includes three beams 50, 50', 50". Any number of beams, alternatively, can be utilized to construct a modular structural section 30 of the bridge 20 depending on desired width span on load requirements. Each of the beams 50, 50', 50" in the bridge 20 is generally identical in length, width and depth. However, beams of different lengths and or widths can be utilized in the modular structural section 30 of the bridge of the present invention. Alternative embodiments of the beam 50 can be seen in related, commonly assigned Modular Composite Support Structure applications referenced previously.

As shown in FIG. 5, each of the beams 50 comprise lateral flanges 51, 52 which are positioned on and supported by one of the two support members 22. Each of the beams 50 has a medial web 53 between and extending below the flanges 51, 52. The medial web 53 includes a inclined sidewall 54 angled generally diagonally with relation to the lower face sheet 40 (FIGS. 4-6). The flanges 51, 52 and the medial web 53 extend longitudinally along the length of the beams 50. The configuration of the flanges and the medial web can take a variety of configurations in alternative embodiments.

The flanges 51, 52 of the beams 50 are spaced apart, and each has a generally planar upper surface 57, 58. The upper surfaces 57, 58 contact the lower facesheets 40 to provide support thereto. The upper surfaces 57, 58 of each flange 51, 52 also provide a surface for bonding or bolting the beam 50 to the sandwich panel 34. The flanges 51, 52 are generally positioned parallel to the lower surface 42 of the lower facesheet 40 (FIG. 7).

The inclined side walls 54 of the beams 50 extend at an angle from the flanges 51, 52. Preferably, this angle is between about 20° to 35° (preferably about 28°) from the vertical perpendicular to the planar upper surfaces 57, 58 of a respective adjacent flange 51, 52. The beams 50 are designed for simple fabrication and handling.

The medial web 53 also has a flat floor 68 between the inclined side walls 54. The floor 68 extends throughout the length of the beam 50. The floor 68 defines a bottom trough 59 of the flat U-shaped beam 50 (FIGS. 4-5). The flat floor

68 allows the beam 50 to be supported on a support member 22 having a flat portion 25. In an alternative embodiment, a bridge can be constructed by placing the beams 50 on a flat concrete slab supported by the flat floor portions as explained herein. Column supports of various configurations can be added in other alternative embodiments to support the flanges 51, 52.

The fibers in the floor 68 are preferably substantially oriented unidirectionally in the longitudinal direction of the beam 50. Such unidirectional fiber orientation provides this beam 50 with sufficient bending stiffness for shorter spans to meet design requirements, particularly along its longitudinal extent.

The fibers in the inclined side walls 54 of the web 53 are oriented in the optimal manner to satisfy design criteria preferably in a substantially quasi-isotropic orientation. A significant number of ±45° plies are necessary to carry the transverse shear loads.

The inclined side walls 54 and the flat floor 68 provide dimensional stability to the shape of the beam 50 during forming. The flanges 51, 52 and medial web 53 form a U-shaped open cross-section having a flat bottom of the beam 50. The beam 50 is designed to carry multi-direction loads. The inclined side walls 54 transfer load between the deck (compression) and the floor (tension) and distribute the reaction load to the support members. As the beam 50 constitutes an open member, the resulting beam 50 provides torsional flexibility during shipping and assembly. However, when the beam 50 is connected with the deck 32, the combination thereof forms a closed section which is extremely strong and stiff.

As seen in FIG. 4, the flanges 51, 52 of the beams 50 each also have respective lower surfaces 71, 72. The lower surfaces 71, 72 each provide a surface for positioning the beam 50 on the support members 22. In constructing the bridge 20, the beams 50 are positioned on the support members 22 to provide a simply supported bridge (FIGS. 4 and 5).

FIG. 6 illustrates an internal diaphragm 84 inserted in the open trough 25 at each end 55, 56 of the beam 50. The diaphragm 84 is preferably formed of a polymer matrix composite material as described herein and shown in FIG. 6. Alternatively the diaphragm 84 can be provided of a variety of structural materials including steel, wood and concrete. The diaphragm 84 increases the torsional stability of the beam 50 for handling and maintains wall stability during installation.

FIGS. 17-19 illustrate alternative diaphragms. FIG. 17 illustrates a plurality of internal diaphragms 170 each having a periphery shaped to matingly contact the contoured shape of the internal trough 25 of the beams 50 when inserted therein in the modular structural section 30. A plurality of external diaphragms 172 is also provided. Each external diaphragm 172 has a periphery shaped to matingly contact the exterior surface 85 of adjacent beams 50, 50'. The diaphragm 170 is inserted into the interior of the beam. The diaphragms 172 are each inserted in the cavity formed between the exterior surfaces 85, 85' of the beams 50, 50'.

The diaphragms 170, 172 are preferably formed of a polymer matrix composite material. Alternatively the diaphragm 170, 172 can be provided of a variety of structural materials including steel, wood and concrete. The diaphragms 170, 172 increase the torsional stability of the beams 50, 50' for handling and maintains wall stability during installation.

FIGS. 18 and 19 illustrate external face diaphragms 181 and 191 respectively. Diaphragm 181 is includes a generally

rectangular periphery having an upper and lower edge 182, 183 and vertical edges 184, 185 generally sized and configured to correspond to the width and height profile of the modular structural section 30 (FIG. 18). A face 186 of the diaphragm 181 is connected to the end of modular structural section 30. The vertical edges 184, 185 extend beyond the inclined side walls 54 of the beams 50, 50" a distance generally equal to the width of the modular structural section 30 defined by the edges 90, 91 of the modular structural section 30.

Alternatively, the diaphragm 191 includes a periphery having an upper and lower edge 192, 193 and vertical edges 194, 195 generally sized and configured to correspond to the width and height profile of the modular structural section 30 (FIG. 19). The vertical edges 194, 195 are contoured to correspond to the shape of the flange 51 and inclined side wall 54 of the outermost beams 50, 50". The diaphragm 191 is connected with the end of the modular structural section 30.

The diaphragms 181, 191 are preferably formed of a polymer matrix composite material. Alternatively the diaphragms 181, 191 can be provided of a variety of structural materials including steel, wood and concrete. The diaphragms 181, 191 increase the torsional stability of the beams 50, 50' for handling and maintains wall stability during installation.

The diaphragms 170, 172, 181 and 191 are each preferably connected with the modular structural section 30 by bonding means such as an adhesive. Alternatively, the diaphragms 170, 172, 181 and 191 can be connected with the modular structural section 30 by mechanical fastening means, including but not limited to bolts, screws, or clamps or a combination of mechanical fastening means and bonding means.

Returning to the bridge 20 of FIGS. 1-5, and 7, the U-shaped, flat bottom beams 50 are supported at opposite ends 55, 56 by the support members 22. The U-shaped beams 50 have sufficient strength, rigidity and torsional stiffness that they are provided unsupported in the center portion 69 between the ends 55, 56 supported by the support members 22. Alternatively, the beams can be supported at a variety of interior locations if desired or depending on the requirements of the span length.

The beams 50, 50', 50" are also positioned horizontally adjacent one another on the support members 22. The flanges 51, 52 of each beam 50 each have an outer edge 74. As illustrated in FIG. 5, adjacent outer edges 74, 74' of adjacent beams 50, 50' preferably form a butt joint 76. As shown in FIG. 5, the flanges 51', 52 of adjacent beams 50, 50' are preferably butt joined such that the flanges do not extend over or overlap each other with the medial web 53 of adjacent support webs 53, 53'. Alternatively, other joints can be provided including joints where the flanges overlap adjacent flanges without overlapping the medial portions of the beam.

Alternative shapes and configurations of the beam 50 can be provided. Alternative embodiments of the beam 50 can be seen in the related, commonly assigned Modular Composite Support Structure applications, previously referenced.

Each beam 50 in the bridge 20 is hand laid using heavy knit weight knitted fiberglass fabric. The beam 50 can be formed on a mold which has a shape corresponding to the contour of the beam 50. Hand layup methods are well-known to one of ordinary skill in the art and the details therefore need not be discussed herein. Alternatively, each beam 50 can be fabricated by automated layup methods.

The fabric used in the inclined side walls 54, 58 is a four-ply quasi-isotropic fabric and polyester resin matrix. The beam 50 can be fabricated to a predetermined thickness using hand layup or other method. An additional layer of a predetermined thickness of unidirectional reinforcement fiberglass is preferably added to the floor of the beams 50 interspersed between quasi-isotropic fabrics to further increase their bending stiffness. The total thickness of the beams 50 can vary across a range of thicknesses. The thickness of the beam is preferably between about 0.5 inches and 3 inches. The inclined side walls 54 and flat floor 68 provide dimensional stability to the shape of the beam 50 during forming.

The beams 50 of the bridge 20 therefore provide an improvement over prior concrete and steel beams, which are extremely rigid and can permanently deform or crack if subjected to torsional stress or loads during shipping.

As explained with respect to the core 45 and the upper and lower facesheets 35, 40, the beams 50 can alternatively be fabricated by other methods such as pultrusion, resin transfer molding (RTM), vacuum curing and filament winding and other methods known to one of skill in the art of composite fabrication, the details of which are thereby not discussed herein.

Being formed of polymer matrix composite materials, each of the beams 50 shown in FIGS. 1-5, and 7 weighs under 3600 pounds for a 30 foot span design. Beams 50 can, alternatively, be provided with appropriate weights corresponding to the applicable span, width and space.

In constructing the bridge 20 of the embodiment of FIG. 1, the lateral flanges 51, 52 of the beams 50 are positioned on adjacent peak portions 23 of the support members 22. The medial web 53, including the inclined side walls 54 and the flat floor 68, are positioned and supported in the trough portions 25 of the beams 50. The contoured shape of the support members 22 which corresponds to and matingly joins with the contoured shape of the beams 50 provides stability to the components under load, prevents lateral shifting and facilitates load transfer from the deck through the beams and support members. The beams 50 are also preferably provided with longitudinal ends 55, 56 configured to overlapingly join and thereby secure longitudinally adjacent beams 50, 50'. Therefore, bridges and support structures of various spans, including spans longer than the beams 50, can be constructed by joining beams end-to-end in this fashion. If, alternatively, overlap joints are utilized, the overlap would be fastened with an adhesive as by mechanical means. The joints could also be formed with an inherent interlock in the lap joints.

As shown in FIGS. 1, 2 and 5, the deck 32 is positioned above such that it generally coextensively overlies the upper surfaces 58, 57' of the adjacent flanges 51, 51'. The deck 32 is also positioned generally parallel with the upper surfaces 57, 57', 58, 58' of the flanges 51, 51', 52, 52' thereby providing a surface for bonding or bolting the beams to the deck.

The deck 32 is connected with the beams 50 by inserting bolts 80 through holes 66 through the lower facesheet 40 and 60 through holes 78 through the flanges 51, 52 (FIGS. 5-7). The bolts 80 are then fastened with nuts 81 or other fastening means. The bolts 80 preferably are inserted in holes 78 which extend along the span of the flanges 51, 52 at intervals of approximately two feet. At the ends 55, 56 of the beams 50 the spacing of the bolts 80 is preferably reduced to about one foot. A row of bolts 80 is preferably inserted through each flange 51, 51', 52, 52' of adjacent beams 50, 50'.

To position and access the bolts 80 for securing, holes 79 are formed through the upper facesheet 35 and upper surface 47 of the tubes 46. These holes 79 have a predetermined diameter sufficient to allow for insertion of the bolts into the hollow center of the tubes 46. These holes 79 are also aligned with holes 66, 78 in the lower facesheet 40 and the flanges 51, 52.

In addition to bolting, the flanges 51, 52 and the deck 32 are also preferably bonded together using an adhesive such as concrehesive paste or like adhesives. Thus, a combination adhesive and mechanical bond is preferably formed between the beams 50, 50', 50" and the deck 32.

Alternatively, other connecting means can be provided for connecting the deck to the beams including other mechanical fasteners such as high strength structural bolts and the like. The deck and beams can alternatively be connected with only bolts or adhesives or by other fastening.

Also, as illustrated in FIG. 1, the bridge 20 preferably is provided with a wear surface 21 added to the upper surface 75 of the deck 32. The wear surface 21 is formed of polymer concrete or low temperature asphalt. Alternatively, the wear surface can be formed of a variety of materials including concrete, polymers, fiber reinforced polymers, wood, steel or a combination thereof, depending on the application.

In order to construct the bridge 20 referenced in FIG. 1, support members 22 including peaks 23 are each provided and positioned at a predetermined position and distance depending on the span. Adjacent peaks 23 are laterally positioned a predetermined distance apart corresponding to the distance of separation between the flanges 51, 52 of the beams 50, 50', 50". The support members 22 are also positioned longitudinally a predetermined distance apart equal approximately to the length of the separation of the ends 55, 56 of the beams 50, 50', 50" which are to be supported.

As shown in FIGS. 4 and 5, the beams 50 are then positioned on the support members 22. The lateral flanges 51, 52 of each beam 50 are positioned on and supported by adjacent vertical columns 31 of the support members 22 as described. Further, each longitudinal end 55, 56 of the beams 50, 50', 50" is positioned on and supported by a support member 22. Likewise, the medial web 53 of each beam 50 is then positioned in adjacent trough portions 25. Adjacent flanges 52 and 51' of adjacent beams 50 and 50' are positioned adjacent one another on a single peak 23.

Adjacent sandwich panels 34, 34' are then positioned and lowered onto the beams 50, 50', 50". The sandwich panels 34 are also aligned next to adjacent sandwich panels 34' and connected with the shear key lock 67 or other connecting means as described above. The deck 32 is preferably aligned with the beams 50, 50', 50" such that the longitudinal ends of the deck 32 are positionally aligned with the ends defining the length of the beams 50. Likewise, the edges 86, 87 defining the width of the deck 32 are preferably aligned above the outside edges 88, 89 of the beams 50 defining the width of the three beams 50, 50', 50".

The deck 32 is then fastened to the beams 50 as described above using adhesives, fasteners, including, but not limited to bolts, screws or the like, other connecting means or some combination thereof. After aligning and connecting each of the sandwich panels 34, 34', 34", the deck 32, as shown in FIG. 1, is then completed. The bridge 20 includes a concrete guard rail 82 along each side of the length of the span.

Alternatively, guard rails, walkways, and other accessory components can be added to the bridge. Such accessory components can be formed of the polymer matrix composite

materials as described herein or other materials including steel, wood, concrete or other composite materials.

An alternative embodiment of the support structure in the form of bridge 100 including the modular structural section 30 according to the present invention is shown (FIGS. 9-10). The bridge 100 includes the modular structural section 30 described herein and illustrated in FIG. 2 and support members 101. Like reference numerals with respect to the modular structural section 30 of FIGS. 1-2 are included in FIGS. 9-10.

The support members 101 are precast concrete abutments having a generally flat upper surface 102 (FIGS. 9-10). A load pad 105 is positioned with its lower surface 106 in a predetermined location on the upper surface 102 of the support member 101. Each of the support beams 50, 50', 50" is positioned with the lower surface 70 of the flat floor 68 generally above the upper surface 108 of the load pad 105 (FIG. 10). The load pads 105 absorb load to protect the support member 101 from scratching, cracking or other failure caused by the load of the modular structural section 30.

The modular structural section 30 is positioned with its end 87 generally above the middle portion of the upper surface 102 of the support member 101 in the direction of the span of the bridge 100 (FIG. 9). An adjacent modular structural section 30 can be placed on the flat support member 101 in alternative embodiments. Further alternatively, the modular structural section 30 can be positioned in other positions on the upper surface 102 of the support member 101 such as with the end 87 generally above the edge 103 of the support member 101. The support member 101, also alternatively, can be positioned at any location along the span of the modular structural section 30 as described with respect to the embodiment of the bridge 20 in FIGS. 1-2.

The flanges 51, 52 of the beams 50, 50', 50" are connected with the deck 32 as described herein. The flanges 51, 52 are not in contact with the support member 101 in this embodiment (FIGS. 9-10).

The support member 101, in alternative embodiments, can be formed of other materials including, but not limited to polymer matrix composite and other composite materials, wood, steel and other materials.

FIGS. 13-14 illustrate a further alternative embodiment of the structural support according to the present invention in the form of bridge 120. The bridge 120 includes a modular structural section 130 and support members 101. The support members 101 are those of bridge 100 illustrated in FIGS. 9-10, the description of which is hereby incorporated by reference. The modular section 130 includes the deck 32 as described herein with respect FIGS. 1-2 and beams 150, 150', 150" having a U-shape including a curved floor 168. Like reference numerals with respect to the deck 32 of FIGS. 1-2 are included in FIGS. 13-14. The beam 150 is described in detail in the "Modular Composite Support Structure" application previously referenced and incorporated by reference herein.

A load pad 105 is positioned with its lower surface 106 in a predetermined location on the upper surface 107 of the support member 101 (FIG. 14). Each of the support beams 150, 150', 150" is positioned with the lower surface 151 of the curved floor 168 generally above the upper surface 108 of the load pad 105 (FIG. 14).

The modular structural section 130 is positioned with its end 87 generally above the middle portion of the upper surface 102 of the support member 101 in the direction of

the span of the bridge 120 (FIG. 14). Alternatively, the modular structural section 30 can be positioned in the various locations described with reference to the embodiment of FIGS. 9–10.

Like the embodiment of FIGS. 9–10, the flanges 151, 152 of the beams 150, 150', 150" are connected with the deck 32 as described with respect to the modular structural section 30 herein. The flanges 151, 152 are not in contact with the support member 101 in this embodiment (FIG. 13).

Alternatively, depending of the curvature of the radius of the curved floor 168, a stabilizing member or other stabilizing means for stabilizing the beam on the support member 101 can be positioned adjacent the beam 50 and the support member 101 in alternative embodiments. Suitable stabilizing means include, but are not limited to, members which would stabilize the curved floor 168 by wedging, cradling, or receiving the beam 150. Further alternatively, the support member 101 can be formed having a contoured shape to receive the beam 150 similar to the contoured support member 22 illustrated and described with reference to FIGS. 1 and 2.

An additional embodiment of a support structure in the form of bridge 110 is provided having the modular deck 32 and beams 50, 50', 50" of bridge 20 as described herein with an L-shape support member 111 (FIGS. 11–12). The L-shape support member 111 is a precast concrete abutment. The support member has a lower ledge 112 disposed generally horizontally and a vertical wall 114 generally perpendicular to the lower ledge 112. The lower ledge 112 and the vertical wall 114 form a v-shape configured to receive the modular structural section 30.

Each of the load pads 105, as previously described, is positioned with its lower surface 106 in a predetermined location on the lower ledge 112 of the support member 111 (FIG. 12). Each of the support beams 50, 50', 50" is positioned with the lower surface 70 of the flat floor 68 generally above the upper surface 108 of the load pad 105 (FIG. 12).

The modular structural section 30 is positioned with its end 87 generally contacting the vertical wall 114. Thus, the modular structural section 30 is positioned within the v-shape of the support member 111 providing stability to the modular section 30 (FIGS. 11–12).

Depending of the span of the bridge or other structure a support member 111 can be utilized at each end of the modular structural section 30 or span of the bridge. The upper ledge 115 is preferably below the level of the wear surface 21 of the deck 32.

In bridge 110, The flanges 51, 52 of the beams 50, 50', 50" are connected with the deck 32 as described herein. The flanges 51, 52 are not in contact with the support member 111 in this embodiment.

The support member 111, in alternative embodiments, can be formed of other materials including, but not limited to polymer matrix composite and other composite materials, wood, steel, and other materials.

In a still further embodiment, a bridge 140 is provided (FIGS. 15–16). The bridge 140 has the modular structural section 130 described with respect to FIGS. 13–14 and the support member 111 described and illustrated in FIGS. 11–12. Each of the load pads 105, as previously described, is positioned with its lower surface 106 in a predetermined location on the lower ledge 112 of the support member 111 (FIG. 16). Each of the support beams 150, 150', 150" is positioned with the curved floor 168 generally above the upper surface 108 of the load pad 105 (FIG. 16).

The modular structural section 130 is positioned with its end 187 generally contacting the vertical wall 114. Thus, the modular structural section 130 is positioned within the v-shape of the support member 111 providing stability to the modular section 130 (FIGS. 11–12).

Depending of the span of the bridge or other structure a support member 111 can be utilized at each end of the modular structural section 130 or span of the bridge. The upper ledge 115 is preferably below the level of the wear surface 121 of the deck 132.

In bridge 140, The flanges 151, 152 of the beams 50, 50', 50" are connected with the deck 132 as described herein. The flanges 151, 152 are not in contact with the support member 111 in this embodiment.

The support member 111, in alternative embodiments, can be formed of other materials including, but not limited to polymer matrix composite and other composite materials, wood, steel, and other materials.

Returning to the embodiment illustrated in FIGS. 1–5 and 7, bridge 20 can also be provided as a kit comprising at least one modular structural section 30 having a deck 32 including at least one sandwich panel 34 and at least one beam 50 and, preferably, connecting means for connecting the deck 32 and the beams 50. Such a kit can be shipped to the construction site. Alternatively, a kit for constructing a support structure can be provided comprising at least one modular structural section having at least one sandwich panel configured and formed of a material suitable for constructing a support structure without necessitating a beam.

The use of the bridge 20 in remote terrains (e.g., timber, mining, park or military uses) is facilitated by such kits which can have components including modular structural sections 30 having a deck 32 including sandwich panels 34 and at least one beam 50, which each can be sized to have dimensions less than a variety of dimensional limitations of various transportation modes including trucks, rail, ships and aircraft. For example, the beam 50 and sandwich panel 34 can be sized with dimensions to fit within a standard shipping container having dimensions of 8 feet by 8 feet by 20 feet. Further, the components can alternatively be sized to fit into trailers of highway trucks which have a standard size of up to a 12 foot width. Moreover, such a kit can be provided having dimensions which would fit in cargo aircraft or in boat hulls or other transportation means. Further, the components, including, but not limited to, the U-shaped beam 50 and sandwich panel 34, can be provided as described which are stackable within or on top of another to utilize and maximize shipping and storage space. The light weight of the components of the modular structural section 30 also facilitates the ease and cost of such transportation.

The lightweight modular components of the modular structural section 30 also facilitate pre-assembly and final positioning with light load equipment in constructing the bridge. As described, the bridge 20 of the present invention can be easily constructed. For example, for a 30 foot span bridge 20, a three man crew utilizing a front end loader or forklift and a small crane can construct the bridge in less than five to ten working days. As compared to bridges constructed by conventional steel and concrete materials, the highway bridge 20 is approximately twenty percent of the weight of a similar sized bridge constructed from conventional materials. Structurally the bridge 20 also provides a traffic bearing highway bridge designed to reduce the failure risk by providing redundant load paths between the deck and the supports. Further, the specific stiffness and strength far

exceed bridges constructed of conventional materials, in the embodiment shown in FIGS. 1-7 being approximately as much as 60 per cent greater than conventional bridges.

The bridge 20 of the present invention can also be constructed to replace an existing bridge, and thereby, utilize the existing support members of the existing bridge. Prior to performing the steps of constructing a bridge described above, the existing bridge span of an existing bridge must be removed, while retaining the existing support members. The at least one beam 50 can then be placed on the existing support members and the bridge 20 constructed as described. Alternatively, additional support members can be positioned or cast on the existing supports and the bridge then constructed according to the method described herein. Alternative methods of constructing a bridge according to the present invention can be seen in the related Modular Composite Support Structure applications previously referenced.

Further, the modular structural section 30 or its components including the beam 50 or deck 32 can be used to also repair a bridge. An existing bridge section can be removed and replaced by a modular structural section 30 or component of the beam 50 or deck 32 as described. Further, a bridge 20, once constructed, can be easily repaired by removing and replacing a modular structural section 30, sandwich panel 34 or beam 50. Such repair can be made quickly without extensive heavy machinery or labor.

The bridge 20 of the present invention also can be provided with a variety of widths and spans, depending on the number, width and length of the modular structural sections 30. A bridge span is defined by the length of the bridge extended across the opening or gap over which the bridge is laid. Thus, the configuration of the modular structural section 30, with its sandwich panel 34 and beam 50, provides flexibility in design and construction of bridges and other support structures. For example, in alternative embodiments, a single sandwich panel may be supported by a single or multiple beams in both the span and width directions. Likewise, a single beam may support a portion or an entirety of one of more sandwich panels. Also, the length and width of the separate sandwich panels 34 need not correspond to the length and width of the beams 50 in a modular structural section 30 of the bridge 20 constructed therefrom. Alternatively, a variety of number of sandwich panels can be utilized to provide the desired span and width of the bridge.

Adjacent sandwich panels 34, 34' can be joined longitudinally in the direction of the span of the bridge 20, as shown in FIG. 1, and/or laterally in the direction of the width of the bridge. As such, a bridge also can be provided with a variety of lanes of travel.

As the beams 50 can also be supported at a variety of locations along their length, the bridge span is not limited by the length of the beams. The span of the bridge 20 shown in FIG. 1 coincides with the length of the beams 50. However, beams, in other embodiments, are provided which can be joined with adjacent beams longitudinally to form a bridge having a span comprising the sum of the lengths of the beams.

The bridge 20 of the present invention is a simply supported bridge which is designed to meet AASHTO specifications as previously incorporated by reference herein. As such, the bridge meets at least specific AASHTO standards and other standards including the following criteria. The bridge supports a load of one AASHTO HS20-44 Truck (72,000 lb) in the center of each of four lanes. The

bridge also is designed such that the maximum deflection (in inches) under a live load is less than the span divided by 800. The allowable deflection for a 60 foot span would be less than 0.9 inches. Further, the bridge meets California standards that for simple spans less than 145 feet, the HS load as defined by AASHTO standards produce higher moment and deflection than lane or alternative loadings.

The bridge 20 is also designed to meet certain strength criteria. The bridge 20 has a positive margin of safety using a "first-ply" as the failure criteria and a safety factor of 4.0, which is commonly used in bridge construction to account for neglected loading, load multipliers, and material strength reduction factors. A positive margin of safety is understood to one of ordinary skill in the art, and the details are therefore not discussed herein.

Further, the bridge is designed and configured such that its buckling eigenvalue (E.V.)  $\alpha/FS > 1$ , wherein (E.V.) is the buckling eigenvalue,  $\alpha$  is the knockdown factor of said modular structural section, and FS is the factor of safety. Such buckling considerations are also known to one of ordinary skill in the art and therefore not discussed in detail herein.

In the bridge shown in FIGS. 1-7, shear loads must be transmitted between the web 53 and flanges 51, 52 of the beams 50, 50', 50" and the sandwich panels 34, 34' of the deck 32. This load transfer is achieved in this embodiment of the bridge 20 by bolting. The maximum expected shear load is approximately 4,000 lbs., while the capacity exceeds 17,000 lbs. The deformation and fracture behavior appears ductile leading to load redistribution to surrounding bolts rather than catastrophic failure. Being made of a polymer matrix composite material which is environmentally resistant to corrosion and chemical attack, the sandwich panels 34, as well as the beams 50 can also be stored outdoors, including on site of the bridge 20 construction, without deterioration or environmental harm. The sandwich panels 34 and the beams 50 are preferably gel coated or painted with an outer layer containing a UV inhibitor. Further, the sandwich panels 34 and the beams 50 can be utilized in applications in corrosive or chemically destructive environments such as in marine applications, chemical plants or areas with concentrations of environmental agents.

The invention will now be described in greater detail in the following non-limiting example.

#### EXAMPLE 1

A trapezoidal tube deck for a 30 ft bridge of the configuration generally as described with respect to FIGS. 1-7 was constructed. The deck included sandwich panels which are 7.5 feet in length in the direction of the span of the bridge and 15 feet in width in the direction transverse to the span. The bridge was simply supported at the ends of the 30 foot span. The deck was designed to have a maximum depth limit of 9 inches with a 0.75 inch polymer concrete wear surface bonded to the top of the deck, leaving 8.25 inches for the sandwich panel.

The sandwich panels were constructed comprising a 6.5 inch deep E-glass/Vinylester trapezoidal tube with facesheets of a hybrid of E-glass and carbon fibers. The trapezoidal tubes were made by hand lay-up. The tubes had a 0.25 inch thick trapezoidal section of 80 percent  $\pm 45^\circ$  fabric with 20 per cent 0° tow fibers. In addition, a 0.25 inch floor of 100 per cent 0° fibers was applied to the top and bottom surfaces. The hand lay-up tubes had a fiber volume of about 40 per cent.

The facesheets contained a hybrid of E-glass and graphite. A 0.136 inch layer of quasi-isotropic E-glass was placed on

the outer surface of the facesheets. The facesheet thickness was 0.5 inches. The layup had 42 per cent graphite and 58 percent glass to provide a satisfactory stiffness.

A wheel load was applied in a deck section in using a hydraulic load frame according to AASHTO 20-44 standards. An entire axle load of 32 kips must be carried by a side 7.5 foot long panel without any contribution from an adjacent panel. Each wheel load is 16 Kips. The wheel load is spread over an area of approximately 16 inches by 20 inches which is the size of a double truck tire footprint.

An ABACUS model was used to generate plots of the stresses in all directions in the critical region.

The bridge meets the margin of safety defined as

$$MS = \frac{\text{Allowable Stress}}{\text{Applied Stress}} - 1$$

with a positive margin of safety indicating no failure at the design load.

The critical condition for this deck is interlaminar shear. The failure is interlaminar shear in the corner between the diagonal member and the top surface. This failure will occur at 2.28 times the 32 Kips axle load or about 73 Kips.

The deck was designed to maintain a bending stiffness no less than 80 Kips/inch which is the stiffness of an equivalent concrete slab. The deck also was designed to withstand an ultimate design load of 90 Kips which is approximately two (2) times the AASHTO traffic wheel load specifications.

#### EXAMPLE 2

A second trapezoidal tube deck for the 30 ft. bridge described in Example 1 was also constructed. The deck was of a similar configuration as the deck described in Example 1, except the facesheets were all E-glass fibers instead of the hybrid deck of Example 1. The facesheets were 0.85 inch thick with a layup of 0/45/90/-45.

The upper and lower facesheets were each fabricated with alternating layers of quasi-isotropic and unidirectional knitted fabric. The upper facesheet included a construction of multiple plies. The upper facesheet included a lower ply of 52 oz quasi-isotropic fabric, a middle layer of 3 plies of 48 oz unidirectional fabric and an upper layer of 12 plies of 52 oz quasi-isotropic fabric.

The lower facesheet likewise included a construction of multiple plies. The lower facesheet included an upper ply of 52 oz. quasi-isotropic fabric, a middle layer of 3 plies of 48 oz. unidirectional fabric and a lower layer of 12 plies of 52 oz. quasi-isotropic fabric. The outer quasi-isotropic plies provide durability while the unidirectional plus odd stiffness and strength.

Under the same load conditions as Example 1, the critical condition for the E-glass deck is also interlaminar shear. The critical limitation is this deck is also interlaminar shear. In this deck the failure occurs first in the top section of the pultrusion at the interface between the top of the pultrusion and the diagonal member. The failure will occur at 2.51 times the 32 Kips load or about 80 Kips.

The deck was also designed to maintain a bending stiffness no less than 80 Kips/in which is the stiffness of an equivalent concrete slab. The deck also was designed to withstand an ultimate design load of 90 Kips which is approximately two (2) times the AASHTO traffic wheel load specifications.

The deck exhibited consistent stiffness of 85 Kips/in under cyclic loading up to 180 kips. The deck also withstood

218 kips which is the maximum limit of the load fixture before showing a drop in stiffness to 79 kips/inch.

In the drawings and specification, there has been set forth a preferred embodiment of the invention and, although specific terms are employed, the terms are used in a generic and descriptive sense only and not for purposes of limitation, the scope of the invention being set forth in the following claims.

That which is claimed:

1. A high load bearing support structure comprising:  
at least one modular structural section; and  
support means having a surface having a predetermined contoured shape for supporting said at least one modular structural section,

at least one oblong beam having a pair of lateral flanges and a medial web between said pair of lateral flanges, said pair of lateral flanges and said medial web having a predetermined shape adapted to mate with a predetermined shape of a surface of said support means, each flange of said pair of lateral flanges and said medial web positioned on and supported by said support means, said at least one oblong beam being formed of a polymer matrix composite comprising reinforcing fibers and a polymer resin, a portion of said fibers on a floor portion of said medial web being unidirectionally oriented between longitudinally opposite ends of said at least one oblong beam,

wherein said at least one oblong beam is a unitary structure, and

a load bearing deck mounted to said at least one oblong beam,

wherein said at least one oblong beam provides primary longitudinal support in said high load bearing support structure; and

wherein said at least one oblong beam transfers load from said deck to said support means.

2. A high load bearing support structure as defined in claim 1, wherein said medial web of said at least one oblong beam extends below said pair of lateral flanges.

3. A high load bearing support structure as defined in claim 1, wherein said medial web of said at least one oblong beam has spaced-apart inclined side walls and a floor therebetween, said spaced-apart inclined side walls and said floor forming a U-shape of said at least one oblong beam; and

wherein said predetermined contoured shape of said surface of said support means has a plurality of spaced apart peak portions and a plurality of trough portions positioned adjacent opposite sides of said peak portions.

4. A high load bearing support structure as defined in claim 1, wherein said load bearing deck comprises:

at least one sandwich panel including:  
a core including a plurality of elongated core members having side walls positioned generally adjacent one another;  
an upper facesheet having a lower surface;  
a lower facesheet having an upper surface;  
said elongated core members being sandwiched between and connected with said lower surface and said upper surface.

5. A high load bearing support structure as defined in claim 4, wherein said at least one sandwich panel comprises a plurality of interconnected sandwich panels.

6. A high load bearing support structure as defined in claim 4, wherein at least one of said upper facesheet, said

lower facesheet and said core members is formed of a polymer matrix composite material comprising reinforcing fibers and a polymer resin.

7. A high load bearing support structure as defined in claim 1, wherein said support means are connected with said at least one modular structural section, such that said support structure is a simply-supported support structure.

8. A high load bearing support structure as defined in claim 1 wherein said at least one oblong beam and said surface of said support means are formed of a polymer matrix composite material comprising reinforcing fibers and a polymer resin.

9. A high load bearing support structure as defined in claim 1, further comprising a wear surface overlying an upper surface of said deck for withstanding foot and vehicular traffic.

10. A high load bearing support structure as defined in claim 1, wherein said high load bearing support structure has a span of 60 feet, said high load bearing support structure has a maximum deflection in inches under a predetermined load of 72000 pounds per lane less than or equal to 0.9 inches.

11. The high load bearing support structure of claim 1, wherein a first of said at least one oblong beam is positioned horizontally in contact with a second of said at least one oblong beam.

12. The high load bearing support structure of claim 1, wherein a first flange of a first of said at least one oblong beam overlaps a second flange of a second of said at least one oblong beam.

13. A high load bearing support structure as defined in claim 1, wherein said reinforcing fibers in said polymer matrix composite material are knitted to form a fabric of at least one ply.

14. A modular structural section for constructing a support structure for supporting a high load, said modular structural section comprising:

at least one oblong beam having a pair of lateral flanges and a medial web between said pair of lateral flanges, each flange of said pair of lateral flanges and said medial web having a predetermined shape adapted to mate with a predetermined shape of a surface of at least one support member, each flange of said pair of lateral flanges and said medial web adapted to be positioned on and supported by said at least one support member, said at least one oblong beam being formed of a polymer matrix composite comprising reinforcing fibers and a polymer resin, a portion of said fibers on a floor portion of said medial web being unidirectionally oriented between longitudinally opposite ends of said at least one oblong beam,

wherein said at least one oblong beam is a unitary structure, and

a load bearing deck mounted to said at least one oblong beam,

wherein said at least one oblong beam provides primary longitudinal support in said high load bearing support structure; and

wherein said at least one oblong beam transfers load from said deck to said at least one support member.

15. A modular structural section as defined in claim 14, wherein said medial web of said at least one oblong beam extends below said pair of lateral flanges.

16. A modular structural section as defined in claim 14, wherein said medial web of said at least one oblong beam has spaced-apart inclined side walls and a floor therebetween, said spaced-apart inclined side walls and said

floor forming a U-shape adapted to mate with and connect with said predetermined contoured shape of said surface of said at least one support member including a plurality of spaced-apart peak portions and a plurality of trough portions positioned adjacent opposite sides of said peak portions.

17. A modular structural section as defined in claim 14, wherein said load bearing deck comprises:

at least one sandwich panel including:  
a core including a plurality of elongated core members having side walls positioned generally adjacent one another;  
an upper facesheet having a lower surface;  
a lower facesheet having an upper surface;  
said elongated core members being sandwiched between and connected with said lower surface and said upper surface.

18. A modular structural section as defined in claim 17, wherein said at least one sandwich panel comprises a plurality of interconnected sandwich panels.

19. A modular structural section as defined in claim 17, wherein at least one of said upper facesheet, said lower facesheet and said plurality of elongate core members are formed of a polymer matrix composite comprising reinforcing fibers and a polymer resin.

20. A modular structural section as defined in claim 14, further comprising a wear surface overlying an upper surface of said deck for withstanding foot and vehicular traffic.

21. A modular structural section as defined in claim 14, wherein said modular structural section has a maximum deflection under a predetermined load of 72000 pounds per lane is less than 0.9 inches.

22. A modular structural section as defined in claim 14, wherein said at least one modular structural section is formed of a polymer matrix composite material comprising reinforcing fibers and a polymer resin and said fibers and said resin are selected such that said support structure will have a positive margin of safety under predetermined required lane loads and a predetermined safety factor using a first-ply failure as the failure criteria.

23. A modular structural section as defined in claim 12, wherein said reinforcing fibers in said polymer matrix composite material are knitted to form a fabric of at least one ply.

24. A high load bearing support structure comprising:  
at least one modular structural section; and  
support means having a surface having a generally flat portion for receiving and supporting structures thereon, wherein said at least one modular structural section comprises:

at least one oblong beam having a pair of lateral flanges and a medial web between and extending below said pair of lateral flanges, said medial web having inclined side walls and a floor therebetween, said floor positioned on and supported by said flat portion of said support means, said at least one oblong beam being formed of a polymer matrix composite comprising reinforcing fibers and a polymer resin, a portion of said fibers on said floor being unidirectionally oriented between longitudinally opposite ends of said at least one oblong beam,

wherein said at least one oblong beam is a unitary structure; and

a load bearing deck mounted to said at least one oblong beam,

wherein said at least one oblong beam provides primary longitudinal support in said high load bearing support structure; and

## 27

wherein said at least one oblong beam transfers load from said deck to said support means.

25. A high load bearing support structure as defined in claim 24, wherein said floor includes at least one substantially flat portion, said at least one substantially flat portion positioned on and supported by said generally flat portion of said support means. 5

26. A high load bearing support structure as defined in claim 24, wherein said floor includes at least one substantially curved portion, said curved portion positioned on and supported by said flat portion of said support means. 10

27. A high load bearing support structure as defined in claim 24 wherein each flange of said pair of lateral flanges is positioned on and supported by said support means.

28. A high load bearing support structure as defined in claim 24, wherein said reinforcing fibers in said polymer matrix composite material are knitted to form a fabric of at least one ply. 15

29. A modular structural section for constructing a support structure for supporting a high load, said modular structural section comprising:

at least one oblong beam having a pair of lateral flanges and a medial web between and extending below said pair of lateral flanges, said medial web having inclined side walls adjacent a respective one of said pair of lateral flanges and a floor extending between said inclined side walls, said floor adapted to be positioned on and supported by and contact a flat portion of at least one support member, said at least one oblong beam being formed of a polymer matrix composite comprising reinforcing fibers and a polymer resin, a portion of said fibers on said floor being unidirectionally oriented between longitudinally opposite ends of said at least one oblong beam,

wherein said at least one oblong beam is a unitary structure; and

a load bearing deck mounted to said at least one oblong beam,

wherein said at least one oblong beam provides primary longitudinal support in said high load bearing support structure; and

wherein said at least one oblong beam transfers load from said deck to said at least one support member.

30. A modular structural section as defined in claim 29, wherein said floor includes at least one substantially flat portion, said flat portion positioned on and supported by said flat portion of said at least one support member. 45

31. A modular structural section as defined in claim 29, wherein said floor includes at least one substantially curved portion, said curved portion positioned on and supported by said flat portion of said at least one support member. 50

32. A modular structural section as defined in claim 29, wherein each of said flanges is configured to be positioned on and supported by said at least one support member.

33. A modular structural section as defined in claim 29, wherein said reinforcing fibers in said polymer matrix composite material are knitted to form a fabric of at least one ply. 55

34. A method of constructing a high load bearing support structure comprising:

providing a support member having a surface having a generally flat portion for receiving and supporting structures thereon;

providing at least one modular structural section comprising:

at least one oblong beam having a pair of lateral flanges and a medial web between and extending below said

## 28

pair of lateral flanges, said medial web having inclined side walls and a floor therebetween, said at least one oblong beam being formed of a polymer matrix composite comprising reinforcing fibers and a polymer resin a portion of said fibers on said floor being unidirectionally oriented between longitudinally opposite ends of said at least one oblong beam wherein said at least one oblong beam is a unitary structure; and

mounting a load bearing deck to said at least one oblong beam,

wherein said at least one oblong beam provides primary longitudinal support in said high load bearing support structure; and

wherein said at least one oblong beam transfers load from said deck to said support member.

35. A method of constructing a high load bearing support structure as defined in claim 34, wherein said step of providing at least one modular structural section further comprises:

providing said at least one oblong beam including said floor that includes at least one substantially flat portion; and

positioning said at least one substantially flat portion on said flat portion of said support member.

36. A method of constructing a support structure as defined in claim 34, wherein said step of providing at least one modular structural section further comprises:

providing said at least one oblong beam including a curved floor portion; and

positioning said curved floor portion on said flat portion of said support member.

37. A method of constructing a high load bearing support structure as defined in claim 34, wherein said reinforcing fibers in said polymer matrix composite material are knitted to form a fabric of at least one ply.

38. A modular structural section for constructing a support structure for supporting a high load, said modular structural section comprising:

at least one oblong beam having a pair of lateral flanges and a medial web between said pair of lateral flanges, each flange of said pair of lateral flanges and said medial web having a predetermined shape adapted to mate with a predetermined shape of a surface of at least one support member, each flange of said pair of lateral flanges and said medial web adapted to be positioned on and supported by said at least one support member, wherein said at least one oblong beam is a unitary structure, and

a load bearing deck mounted to said at least one oblong beam, said load bearing deck comprising at least one sandwich panel being an integrally formed, unitary pultruded sandwich panel comprising an upper and a lower facesheet formed by pultrusion and at least one elongate core member formed by pultrusion,

wherein said at least one oblong beam provides primary longitudinal support in said high load bearing support structure; and

wherein said at least one oblong beam transfers load from said deck to said at least one support member.

39. A modular structural section for constructing a support structure for supporting a high load, said modular structural section comprising:

at least one oblong beam having a pair of lateral flanges and a medial web between said pair of lateral flanges,

**29**

each flange of said pair of lateral flanges and said medial web having a predetermined shape adapted to mate with a predetermined shape of a surface of at least one support member, each flange of said pair of lateral flanges and said medial web adapted to be positioned on and supported by said at least one support member, said at least one oblong beam being formed of a polymer matrix composite comprising reinforcing fibers and a polymer resin, a portion of said fibers on a generally inclined side wall of said medial web being in a quasi-isotropic orientation,

wherein said at least one oblong beam is a unitary structure, and

**30**

a load bearing deck mounted to said at least one oblong beam,

wherein said at least one oblong beam provides primary longitudinal support in said high load bearing support structure; and

wherein said at least one oblong beam transfers load from said deck to said at least one support member.

**40.** A modular structural section as defined in claim **39**, wherein said reinforcing fibers in said polymer matrix composite material are knitted to form a fabric of at least one ply.

\* \* \* \* \*